



US008459309B2

(12) **United States Patent**  
**Cronburg et al.**

(10) **Patent No.:** **US 8,459,309 B2**  
(45) **Date of Patent:** **\*Jun. 11, 2013**

(54) **SAILCLOTH WITH HIGH 1% WARP AND HIGH WARP EFFICIENCY AND METHOD OF MAKING SAME**

(75) Inventors: **Terry Lee Cronburg**, Coventry, CT (US); **Robert H. Bainbridge**, West Hartford, CT (US)

(73) Assignee: **Challenge Sailcloth Inc.**, Vernon, CT (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/347,224**

(22) Filed: **Jan. 10, 2012**

(65) **Prior Publication Data**

US 2012/0174848 A1 Jul. 12, 2012

**Related U.S. Application Data**

(63) Continuation of application No. 12/332,262, filed on Dec. 10, 2008, now Pat. No. 8,118,065.

(51) **Int. Cl.**

**D03D 13/00** (2006.01)  
**D03D 7/00** (2006.01)  
**D03D 23/00** (2006.01)  
**D03D 25/00** (2006.01)

(52) **U.S. Cl.**

USPC ..... **139/425 R**; 139/383 R; 139/420 R; 139/420 A; 139/DIG. 1

(58) **Field of Classification Search**  
USPC ..... 139/383 R, 384 R, 386, 420 R, 429 R, 139/420 A, DIG. 1  
See application file for complete search history.

(56) **References Cited**

**U.S. PATENT DOCUMENTS**

3,022,545 A \* 2/1962 Wylde et al. ..... 28/267  
3,626,886 A \* 12/1971 Cafiero ..... 114/102.33  
4,590,121 A \* 5/1986 Mahr ..... 442/185  
4,953,489 A \* 9/1990 Bassett ..... 114/102.33  
5,304,414 A \* 4/1994 Bainbridge et al. ..... 442/208  
6,725,885 B2 \* 4/2004 Mahr ..... 139/383 R  
8,118,065 B2 \* 2/2012 Cronburg et al. ..... 139/426 R  
2002/0164911 A1 \* 11/2002 Cunningham et al. ..... 442/135  
2002/0177377 A1 \* 11/2002 Mahr ..... 442/203  
2003/0111128 A1 \* 6/2003 Hannigan et al. ..... 139/421  
2005/0039662 A1 \* 2/2005 Skinner et al. ..... 114/102.29  
2007/0099526 A1 \* 5/2007 Heerden et al. ..... 442/135

\* cited by examiner

*Primary Examiner* — Bobby Muromoto, Jr.

(74) *Attorney, Agent, or Firm* — Jeremy C. Lowe; Axinn Veltrop Harkrider LLP

(57) **ABSTRACT**

There is provided herein a woven sailcloth having a weight of at least about 6 and comprising warp yarns and fill yarns and having a 1% warp of at least about 80 and/or a warp efficiency of at least about 13, wherein the fill yarns are pre-crimped, and wherein the warp yarns and the fill yarns are weaved in a plain weave in which the ratio of fill yarn count to warp yarn count is about 1.1:1 to about 1.8:1 and the ratio of warp yarn density to fill yarn density is about 1.2:1 to about 1.9:1. There is also provided herein sails made from the sailcloth and a method for making the sail.

**62 Claims, No Drawings**

**SAILCLOTH WITH HIGH 1% WARP AND HIGH WARP EFFICIENCY AND METHOD OF MAKING SAME**

**CROSS-REFERENCE TO RELATED APPLICATIONS**

This application is a continuation of U.S. Ser. No. 12/332, 262 filed Dec. 10, 2008, which is incorporated herein by reference in its entirety.

**TECHNICAL FIELD**

The present disclosure relates to woven sailcloth with high 1% warp and high warp efficiency, as well as a method of making same.

**BACKGROUND OF THE INVENTION**

“Crimp” is a term that is used to describe the waviness or nonlinearity of yarns in woven fabrics. Typically, such yarns have an “over and under” shape caused by weaving. The more crimp that is present in a woven fabric, the more the fabric will stretch. Stretchiness is an important consideration in the selection of a woven fabric as sailcloth. If sailcloth stretches too much, it loses its shape and is aerodynamically inefficient.

The sail-making industry has attempted to address the issue of crimp in a number of ways. For example, sailcloths have been laminated with one or more layers of nonwoven plastic film to minimize stretching of the sailcloth in the wind. Unfortunately, laminated sailcloths delaminate with age, use, and exposure to the elements. In addition, the laminating film tends to crease and shrink with use, thereby adversely affecting the shape of the sail.

Also, in an effort to minimize stretching, sailcloth, which has been tightly woven from polyester yarns, has been impregnated with a resin and heated to cure the resin and shrink the polyester fabric. In order to construct sails from this sailcloth, numerous panels must be assembled to align the yarns with less crimp along directions of maximum stress or load in the sail so as to reduce stretch. Therefore, the disadvantage of this type of sailcloth is that it limits how panels can be cut and arranged in a sail, while still using the sailcloth efficiently.

Sailcloth also has been constructed with a reinforcing yarn to minimize stretching. The reinforcing yarn, which has a higher tensile modulus (e.g., above 500 grams/denier) than conventional yarn (tensile modulus of 20-100 grams/denier for Dacron or polyester), has been used to replace the conventional yarn every so many yarns in the warp and/or fill direction, while maintaining the denier (see, e.g., Bainbridge et al., U.S. Pat. No. 5,304,414). More recently, sailcloths have been proposed that are woven from heat-shrinkable yarn with crimp imparted to the fill yarns, while leaving the warp yarns relatively uncrimped. Such sailcloths have a ratio of warp density to fill density below 0.93:1 (see, e.g., Mahr, U.S. Pat. No. 6,725,885).

More structured sails have been developed for racing. Fabric strips, which contain bundles of monofilaments, have been taped onto the skin or membrane of the sail along the load path in the sail. However, such sails have proved to have insufficient durability. Consequently, structural sails having a complex secondary structure in which the angles of warp yarns with respect to fill yarns vary in one panel relative to another panel have been proposed (see, e.g., Keire, U.S. Pat. No. 6,257,160). Separately, the use of pre-crimped fill yarn has been proposed to allow for warp yarn to remain predomi-

nantly straight with very little crimp (see, e.g., Cronburg, U.S. Pat. App. Pub. No. 2006/0157138).

In view of the above, the present disclosure seeks to provide woven fabric, in particular sailcloth, in which the warp yarns not only remain predominantly straight with very little crimp but also have a high 1% warp and a high warp efficiency. The present disclosure also seeks to provide a method of making same. These and other objects and advantages, as well as inventive features, will become apparent from the 10 detailed description provided herein.

**SUMMARY OF THE INVENTION**

A woven sailcloth comprising warp yarns and fill yarns is 15 provided. The woven sailcloth has a 1% warp of at least about 125 and/or a warp efficiency of at least about 17.

Another woven sailcloth comprising warp yarns and fill 20 yarns is also provided. The warp yarns and fill yarns are weaved in a plain weave in which the ratio of fill yarn count to warp yarn count is about 1.1:1 to about 1.8:1, and the ratio of warp yarn density to fill yarn density is about 1.2:1 to about 1.9:1. The woven sailcloth has a 1% warp of at least about 125 and/or a warp efficiency of at least about 17.

Yet another woven sailcloth comprising warp yarns and fill 25 yarns is provided. The woven sailcloth has a weight of at least about 7 and at least one of: a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1.

Still yet another woven sailcloth comprising warp yarns and fill 30 yarns is provided. The woven sailcloth has a weight of at least about 7. The warp yarns and fill yarns are weaved in a plain weave in which the ratio of fill yarn count to warp yarn count is about 1.1:1 to about 1.8:1, and the ratio of warp yarn density to fill yarn density is about 1.2:1 to about 1.9:1. The woven sailcloth has a 1% warp of at least about 125 and/or a warp efficiency of at least about 17. The woven 35 sailcloth also has at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1.

Further provided is a sail comprising panels of sailcloth at 40 least one of which is woven sailcloth as described herein. Desirably, the at least one panel of woven sailcloth as 45 described herein is assembled into the sail with load paths oriented along its warp yarns.

Still further provided is a method of making a woven sailcloth comprising warp yarns and fill yarns. The method 50 comprises weaving warp yarns and fill yarns in a plain weave in which the ratio of fill yarn count to warp yarn count is about 1.1:1 to about 1.8:1 and the ratio of warp yarn density to fill 55 yarn density is about 1.2:1 to about 1.9:1.

Even still further provided is a method of making a sail. The method comprises assembling panels of sailcloth, at least 60 one panel of which is woven sailcloth as described herein and which is assembled into the sail with load paths oriented along its warp yarns.

**DETAILED DESCRIPTION**

The present disclosure is predicated on the surprising and unexpected discovery that in a heavier woven sailcloth

wherein the warp yarns are predominantly straight with very little crimp the woven sailcloth has a high 1% warp and a high warp efficiency. The woven sailcloth also has other superior characteristics.

The following terms are relevant to the present disclosure:

(a) "Yarn" and "yarns" are used herein to refer to any and all fibers, filaments, strands, and/or yarns of natural, synthetic, or composite (e.g., natural and synthetic) material that can be woven into a fabric, in particular sailcloth.

(b) "Warp" describes a yarn that runs lengthwise in a fabric.

(c) "Weft" describes a yarn that runs widthwise in a fabric. This yarn also may be referred to as a "fill" yarn.

(d) "Woven" describes a fabric that is made by weaving warp and fill yarns together, such as by operation of a loom. The warp and fill yarns cross over and under each other as the fabric is woven.

(e) "Crimp" describes the waviness or nonlinearity of yarns in woven fabrics (see, e.g., *Man-Made Fiber and Textile Dictionary*, Celanese Corporation). Crimp can occur in the warp and/or weft yarns. Factors, such as the relative thickness ("denier") of the yarns and the tension of the yarns, can affect crimp. A thinner yarn (lower denier) will crimp more than a thicker yarn (higher denier). Likewise, a yarn under less tension will crimp more than a yarn under more tension. Crimp can be measured by making gage marks on a woven fabric a set distance apart. For example, marks can be made about one meter apart along the length of the fabric. A warp yarn between two gage marks is then unraveled. The unraveled yarn is straightened out, and its length is measured. The length of the unraveled yarn in excess of the gage (in this example, in excess of one meter) is a measure of the crimp. If, for example, the unraveled warp yarn is 1.15 meters in length, it has a 15% crimp. The crimp in a weft yarn can be similarly measured between gage marks marked on a woven fabric a set distance apart along the width of the fabric.

(f) "Denier" is the weight in grams of a 9,000 meter length of yarn. The denier is proportional to the square of the effective diameter of the yarn.

(g) "Average denier" is  $[(a)(b)+(c)(d)]/(b+d)$ , wherein "a" and "c" are the number of threads of denier "b" and "d," respectively.

(h) "Plain weave" describes a manner of weaving in which warp yarns pass over and under weft (or fill) yarns.

(i) "Ripstop" describes a woven fabric in which a reinforcing yarn has been used at a designated interval, which can vary from one fabric to another and, if desired, within a single fabric. Depending on how the reinforcing yarn is incorporated, the woven fabric can take on a variety of textures, such as a box pattern. The presence of the reinforcing yarn makes the fabric difficult to rip; hence, the term "ripstop."

(j) "Density" of a fabric is determined by multiplying the square root of the yarn in denier by the yarn count per inch.

(k) "Greige" refers to a woven fabric in an unfinished state.

(l) "Bias" refers to the direction of the fabric at 45° from the warp direction or the fill direction.

(m) "1% warp" refers to the amount of weight (in pounds) that must be applied to woven fabric for the warp yarns to stretch or elongate 1%.

(n) "10 lb. warp" is the number of hundredths of an inch that warp yarn elongates under 10 lbs. of force. A 2 inch×16 inch sample of woven fabric is stretched with 10 lbs. of force in the 16-inch direction, and the elongation of the warp yarn is measured.

(o) "10 lb. fill" is the number of hundredths of an inch that fill yarn elongates under 10 lbs. of force. A 2 inch×16 inch

sample of woven fabric is stretched with 10 lbs. of force in the 16-inch direction, and the elongation of the fill yarn is measured.

(p) "10 lb. bias" is the number of hundredths of an inch that woven fabric elongates along its bias under 10 lbs. of force. A 2 inch×16 inch sample of woven fabric, which has been cut along its bias, is stretch with 10 lbs. of force in the 16-inch direction, and the elongation of the fabric is measured.

(q) "50 lb. warp" is the number of hundredths of an inch that warp yarn elongates under 50 lbs. of force. A 2 inch×16 inch sample of woven fabric is stretched with 50 lbs. of force in the 16-inch direction, and the elongation of the warp yarn is measured.

(r) The "weight" of woven fabric is measured in ounces per sailmaker yard, which is 36 inches×28.5 inches.

(s) "Efficiency" is a term used to describe the ability of a woven fabric having a given weight to resist stretching. For example, if a woven fabric resists stretching but weighs a lot, it is considered to be relatively inefficient, or to have low efficiency. By contrast, if a woven fabric resists stretching and does not weigh a lot, it is considered to be relatively efficient, or to have relatively high efficiency.

(t) "Warp efficiency" = 1% warp/weight.

(u) "1% W:1% F" is the ratio of 1% warp to 1% fill.

(v) "1% F:1% B" is the ratio of 1% fill to 1% bias.

(w) "1% W:1% F:1% F:1% B" is the ratio of 1% W:1% F to 1% F:1% B.

(x) "10#W:10#F" is the ratio of 10 lb. warp to 10 lb. fill.

(y) "10#F:10#B" is the ratio of 10 lb. fill to 10 lb. bias.

(z) "10#W:10#F:10#F:10#B" is the ratio of 10#W:10#F to 10#F:10#B.

The above terminology may be used herein to describe one or more aspects of the present disclosure. The terminology is not intended to limit the scope of the claimed invention.

A woven sailcloth comprising warp yarns and fill yarns is provided. The woven sailcloth comprising warp yarns and fill yarns can have a weight of at least about 6, such as 6.39. Accordingly, the woven sailcloth can have a weight of at least about 6.5, at least about 7, at least about 7.5, at least about 8, at least about 8.5, at least about 9, at least about 9.5, or at least about 10. In a preferred embodiment of the invention, the woven sailcloth has a weight of 7.94. In another preferred embodiment of the invention, the woven sailcloth has a weight of 9.78.

In a preferred embodiment, the woven sailcloth has a 1% warp of at least about 125. Accordingly, the woven sailcloth can have a 1% warp of at least about 125, at least about 130, at least about 135, at least about 140, at least about 145, at least about 150, at least about 155, at least about 160, at least about 165, at least about 170, at least about 175, at least about 180, at least about 185, at least about 190, at least about 195, at least about 200, and at least about 205. The woven sailcloth also preferably has a warp efficiency of at least about 17. Accordingly, the woven sailcloth can have a warp efficiency of at least about 17, at least about 18, at least about 19, at least about 20, and at least about 21. In a preferred embodiment, the woven sailcloth has a 1% warp of at least about 125 (e.g., at least about 140) and/or a warp efficiency of at least about 17. In another preferred embodiment, the woven sailcloth has a 1% warp of at least about 190 (e.g., at least about 205) and/or a warp efficiency of at least about 21. Preferably, the woven sailcloth also has at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. bias ratio of less than about

60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325

0.5:1. Preferably, the sailcloth has a weight of at least about 7, more preferably at least about 9. Preferably, the warp yarns and the fill yarns are weaved in a plain weave in which the ratio of fill yarn count to warp yarn count is about 1.1:1 to about 1.8:1, and the ratio of warp yarn density to fill yarn density is about 1.2:1 to about 1.9:1.

In another preferred embodiment, the woven sailcloth comprises warp yarns and fill yarns that are weaved in a plain weave in which the ratio of fill yarn count to warp yarn count is about 1.1:1 to about 1.8:1, and the ratio of warp yarn density to fill yarn density is about 1.2:1 to about 1.9:1. The woven sailcloth has a 1% warp of at least about 125, more preferably at least about 190, and/or a warp efficiency of at least about 17, more preferably at least about 21. The woven sailcloth preferably has a weight of at least about 7, more preferably at least about 9. In addition, the woven sailcloth preferably has at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1.

In yet another preferred embodiment, the woven sailcloth has a weight of at least about 7 and one or more (such as two, three, four, five, six, seven, eight or all) of the following: a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1. Preferably, the woven sailcloth has a 1% warp of at least about 125 (e.g., at least about 140) and/or a warp efficiency of at least about 17; more preferably, the woven sailcloth has a 1% warp of at least about 190 (e.g., at least about 205) and/or a warp efficiency of at least about 21. Preferably, the woven sailcloth has a weight of at least about 9. Preferably, the warp yarns and fill yarns that are weaved in a plain weave in which the ratio of fill yarn count to warp yarn count is about 1.1:1 to about 1.8:1, and the ratio of warp yarn density to fill yarn density is about 1.2:1 to about 1.9:1.

In still yet another preferred embodiment, the woven sailcloth has a weight of at least about 7 and comprises warp yarns and fill yarns weaved in a plain weave in which the ratio of fill yarn count to warp yarn count is about 1.1:1 to about 1.8:1 and the ratio of warp yarn density to fill yarn density is about 1.2:1 to about 1.9:1. The woven sailcloth has a 1% warp of at least about 125 and/or a warp efficiency of at least about 17. The woven sailcloth has at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1. Preferably, the weight of the woven sailcloth is at least about 9, and the woven sailcloth has a 1% warp of at least about 190 and/or a warp efficiency of at least about 21.

The woven sailcloth comprising warp yarns and fill yarns can have a 1% warp to 1% fill ratio of at least about 4.9:1. The 1% warp to 1% fill ratio can be as high as about 24:1, such as 24:1. Accordingly, the woven sailcloth can have a 1% warp to 1% fill ratio of at least about 5:1, at least about 6:1, at least about 7:1, at least about 8:1, at least about 9:1, at least about 10:1, at least about 11:1, at least about 12:1, at least about 13:1, at least about 14:1, at least about 15:1, at least about

16:1, at least about 17:1, at least about 18:1, at least about 19:1, at least about 20:1, at least about 21:1, at least about 22:1, or at least about 23:1.

The woven sailcloth comprising warp yarns and fill yarns can have a 1% fill to 1% bias ratio of less than about 0.8:1, such as 0.74:1. The 1% fill to 1% bias ratio can be as low as about 0.62:1, such as about 0.67:1, or even lower. Accordingly, the woven sailcloth can have a 1% fill to 1% bias ratio of less than about 0.7:1, less than about 0.6:1, or less than 0.5:1.

The woven sailcloth comprising warp yarns and fill yarns can have a 1% warp:1% fill to 1% fill:1% bias ratio of at least about 7:1, such as 7.33:1. The 1% warp:1% fill to 1% fill:1% bias ratio can be as high as about 33:1, such as 32.47:1, or even higher. The 1% warp:1% fill to 1% fill:1% bias ratio can be 21.59:1, for example. Accordingly, the woven sailcloth can have a 1% warp:1% fill to 1% fill:1% bias ratio of at least about 8:1, at least about 9:1, at least about 10:1, at least about 11:1, at least about 12:1, at least about 13:1, at least about 14:1, at least about 15:1, at least about 16:1, at least about 17:1, at least about 18:1, at least about 19:1, at least about 20:1, at least about 21:1, at least about 22:1, at least about 23:1, at least about 24:1, at least about 25:1, at least about 26:1, at least about 27:1, at least about 28:1, at least about 29:1, at least about 30:1, at least about 31:1, or at least about 32:1.

The woven sailcloth comprising warp yarns and fill yarns can have a 10 lb. warp to 10 lb. fill ratio of less than about 0.5:1, such as 0.44:1. The 10 lb. warp to 10 lb. fill ratio can be as low as about 0.07:1, such as about 0.09:1, or even lower. Accordingly, the woven sailcloth can have a 10 lb. warp to 10 lb. fill ratio of less than about 0.4:1, less than about 0.3:1, less than about 0.2:1, less than about 0.1:1, less than about 0.09:1, less than about 0.08:1, less than about 0.07:1, less than about 0.06:1, or less than about 0.05:1.

The woven sailcloth comprising warp yarns and fill yarns can have a 10 lb. fill to 10 lb. bias ratio of at least about 1.1:1, such as 1.12:1. The 10 lb. fill to 10 lb. bias ratio can be as high as about 2.5:1, such as at least about 1.5:1, or even higher. Accordingly, the woven sailcloth can have a 10 lb. fill to 10 lb. bias ratio of at least about 1.2:1, at least about 1.3:1, at least about 1.4:1, at least about 1.5:1, at least about 1.6:1, at least about 1.7:1, at least about 1.8:1, at least about 1.9:1, at least about 2.0:1, at least about 2.1:1, at least about 2.2:1, at least about 2.3:1, at least about 2.4:1 or at least about 2.5:1.

The woven sailcloth comprising warp yarns and fill yarns can have a 10 lb. warp:10 lb. fill to 10 lb. fill:10 lb. bias ratio of less than about 0.4:1, such as 0.39:1. The woven sailcloth can have a 10 lb. warp:10 lb. fill to 10 lb. fill:10 lb. bias ratio of less than about 0.06:1, such as less than about 0.03:1, or even lower. Accordingly, the woven sailcloth can have a 10 lb. warp:10 lb. fill to 10 lb. fill:10 lb. bias ratio of less than about 0.5:1, less than about 0.4:1, less than about 0.3:1, less than about 0.2:1, less than about 0.1:1, less than about 0.09:1, less than about 0.08:1, less than about 0.07:1, less than about 0.06:1, less than about 0.05:1, less than about 0.04:1, or less than about 0.03:1.

Any suitable yarn can be used. Examples of suitable yarns include, but are not limited to, polyester yarn, such as a Dacron-type polyester yarn, and polyamide yarn, such as a nylon yarn. Preferably, the fill yarns are pre-crimped and stretchable (see, e.g., Cronburg, U.S. Pat. App. Pub. No. 2006/0157138, incorporated herein by reference; see also, Smith et al., U.S. Pat. No. 5,771,674 for a method of crimping fibers, also incorporated herein by reference).

The denier of a warp yarn preferably ranges from about 500 to about 1,500. Therefore, the denier of a warp yarn can be

about 550, about 575, about 600, about 625, about 650, about 675, about 700, about 725, about 750, about 775, about 800, about 825, about 850 (such as 840), about 875, about 900, about 925, about 950, about 975, about 1,000, about 1,025, about 1,050, about 1,075, about 1,100, about 1,125, about 1,150, about 1,175, about 1,200, about 1,225, about 1,250, about 1,275, about 1,300, about 1,325, about 1,350, about 1,375, about 1,400, about 1,425, about 1,450, about 1,475, or about 1,500. The denier of a weft/fill yarn preferably ranges from about 150 to about 350. Therefore, the denier of a weft/fill yarn can be about 150, about 155 (such as about 157), about 160, about 165, about 170 (such as about 171.88 or 172), about 175, about 180, about 185, about 190, about 195, about 200, about 205, about 210, about 215, about 220, about 225, about 230, about 235, about 240, about 245, about 250, about 255, about 260, about 265, about 270, about 275, about 280, about 285, about 290, about 295, about 300, about 305, about 310, about 315 (such as about 313.33 or 313), about 320, about 325, about 330, about 335, about 340, about 345, or about 350.

In this regard, the denier of a weft/fill yarn can be achieved by weaving a lower denier yarn in combination with a higher denier yarn such that an effective denier in the preferred range is achieved. For example, a fill yarn of 150 denier can be weaved with a fill yarn of 220 denier. If nine yarns of 150 denier are weaved with one yarn of 220 denier, an effective average denier of 157, which is within the preferred range, can be achieved. Similarly, a fill yarn of 150 denier can be weaved with a fill yarn of 500 denier. If 15 yarns of 150 denier are weaved with one yarn of 500 denier, an effective average denier of 171.88, which is within the preferred range, can be achieved. Similarly, two or more yarns can be combined as a single yarn for weaving. For example, two fill yarns of 150 denier can be weaved together as one, resulting in a denier of 300. The resulting fill yarn having a denier of 300 can be weaved with a fill yarn of 500 denier. If 14 fill yarns of 300 denier are weaved with one fill yarn of 500 denier, an effective average denier of 313.33, which is within the preferred range, can be achieved. One of ordinary skill in the art will readily appreciate that numerous other combinations of deniers and combinations of yarn counts (i.e., number of yarns of one denier woven with number of yarns of another denier) can result in a denier or average denier within the preferred range.

Preferably, the ratio of fill yarn count (yarns/inch) to warp yarn count (yarns/inch) is about 1.1:1 to about 1.8:1. Thus, the ratio of fill yarn count to warp yarn count can be about 1.1:1, about 1.2:1, about 1.3:1, about 1.4:1, about 1.5:1, about 1.6:1, about 1.7:1 or about 1.8:1. The ratio of fill yarn count to warp yarn count can be from about 1.1:1 to about 1.7:1, about 1.1:1 to about 1.6:1, about 1.1:1 to about 1.5:1, about 1.1:1 to about 1.4:1, about 1.1:1 to about 1.3:1, or about 1.1:1 to about 1.2:1.

Preferably, the average warp yarn density is about 1,300 to about 1,700. Thus, the average warp yarn density can be about 1,325, about 1,350, about 1,375, about 1,400, about 1,425, about 1,450, about 1,475, about 1,500, 1,525, about 1,550, about 1,575, about 1,600, about 1,625, about 1,650, about 1,675 or about 1,700.

Preferably, the concurrent average weft/fill yarn density is about 800 to about 1,300. Thus, the average weft/fill yarn density can be about 825, about 850, about 875, about 900, about 925, about 950, about 975, about 1,000, about 1,025, about 1,050, about 1,075, about 1,100, about 1,125, about 1,150, about 1,175, about 1,200, about 1,225, about 1,250, about 1,275 or about 1,300.

Preferably, the ratio of warp yarn density to fill yarn density is about 1:1 to about 2:1. Thus, the ratio of average warp yarn density to average fill yarn density can be about 1:1, about

1.1:1, about 1.2:1, about 1.3:1, about 1.4:1, about 1.5:1, about 1.6:1, about 1.7:1, about 1.8:1, about 1.9:1 or about 2:1. The ratio of warp yarn density to fill yarn density can be from about 1.1:1 to about 1.9:1, from about 1.2:1 to about 1.9:1, from about 1.3:1 to about 1.9:1, about 1.4:1 to about 1.9:1, about 1.5:1 to about 1.9:1, about 1.6:1 to about 1.9:1, about 1.7:1 to about 1.9:1, or about 1.8:1 to about 1.9:1.

The warp yarns and fill yarns can be weaved into any suitable weave. The fill yarns are preferably pre-crimped. A preferred weave is a plain weave. In this regard, it is preferred that a reinforcing yarn (i.e., a yarn of a higher denier) is used with the fill yarn, such as every  $n^{th}$  yarn, wherein "n" is preferably an integer from and including 5 to and including 20, such as 5, 6, 7, 8, 9, 10, 11, 12, 13, 14, 15, 16, 17, 18, 19, or 20. An "n" of 10, 14 or 15 can be preferred. By incorporating a reinforcing yarn, the fill yarns can be weaved in a ripstop pattern, which is preferred.

Preferably, the woven sailcloth is used in the construction of sails. Therefore, provided is a sail comprising panels of sailcloth at least one of which is a panel of woven sailcloth as described herein. The at least one panel of woven sailcloth as described herein is assembled into the sail with load paths oriented along its warp yarns.

Accordingly, also provided is a method of making a woven sailcloth comprising warp yarns and fill yarns. The method comprises weaving warp yarns and fill yarns in a plain weave in which the ratio of fill yarn count to warp yarn count is about 1.1:1 to about 1.8:1 and the ratio of warp yarn density to fill yarn density is about 1.2:1 to about 1.9:1. Preferably, the fill yarns are pre-crimped. The fill yarns preferably comprise a reinforcing yarn. Preferably, the reinforcing yarn is present every  $n^{th}$  yarn, wherein "n" is an integer from and including 5 to and including 20, such as 5, 6, 7, 8, 9, 10, 11, 12, 13, 14, 15, 16, 17, 18, 19, or 20. An "n" of 10, 14 or 15 can be preferred. The fill yarns are preferably weaved in a ripstop pattern.

The woven sailcloth can be finished in accordance with methods known in the art. For example, it can be scoured (e.g., to remove any sizing, wax, dirt, and the like). Afterwards, it can be dipped into an aqueous bath of heat-curable resin, such as melamine, which serves to lock the woven geometry and decrease stretch. The fabric then can be dried and heat-set by passing through an oven or over large, heated, metal cylinders, such as cylinders heated to about 425° F., which causes the yarns to shrink, thereby increasing density. The fabric then can be calendared by passing the fabric between a pair of rollers under high pressure (e.g., 70 tons), with one of the rollers being heated. Instead of being heat-set with melamine, the fabric can be coated with polyurethane or the like. Afterwards, the edges of the fabric are typically slit, and the fabric is tubed off into rolls. These finishing methods are exemplary and are not intended to be limiting.

In view of the foregoing, a method of making a sail is also provided. The method comprises assembling panels of sailcloth, at least one panel of which is woven sailcloth as described herein. The at least one panel of woven sailcloth as described herein is assembled into the sail with load paths oriented along its warp yarns.

## EXAMPLES

The following examples serve to illustrate the present disclosure. The examples are not intended to be limiting.

## Example 1

This example describes a construction of sailcloth referred to as 6.11.

This sailcloth was constructed from 500 denier warp yarn and a mixture of 150 and 220 denier fill yarns. The fill yarns were woven in a repeating pattern of nine 150 denier yarns followed by one 220 denier yarn. This resulted in an average fill denier of 157. The yarns were weaved in a plain weave with a ripstop pattern in the fill yarn.

The griuge fabric contained 62 yarns/inch in the warp and, based on the average fill denier, 85 yarns/inch in the fill. The density of the warp was 1,386, whereas the average density of the fill was 1,065.

The finished fabric contained 75 yarns/inch in the warp, 78.55 yarns/inch in the 150 denier fill, and 8.73 yarns/inch in the 220 denier fill (i.e., a total of 87.28 yarns/inch in the fill). The density of the warp was 1,677, whereas the average density of the fill was 1,093.

## Example 2

This example describes a construction of sailcloth referred to as 8.11.

This sailcloth was constructed from 840 denier warp yarn and 150 and 500 denier fill yarns. The fill yarns were woven in a repeating pattern of 15 150 denier yarns followed by one 500 denier yarn. This resulted in an average fill denier of 171.88. The yarns were weaved in a plain weave with a ripstop pattern in the fill yarn.

The griuge fabric contained 44 yarns/inch in the warp and, based on the average fill denier, 80 yarns/inch in the fill. The density of the warp was 1,275, whereas the average density of the fill was 1,049.

The finished fabric contained 55 yarns/inch in the warp, 78.75 yarns/inch in the 150 denier fill, and 5.25 yarns/inch in the 500 denier fill (i.e., a total of 84 yarns/inch in the fill). The density of the warp was 1,594, whereas the average density of the fill was 1,011.

## Example 3

This example describes a construction of sailcloth referred to as 10.11.

This sailcloth was constructed from 1,500 denier warp yarn and 150 and 500 denier fill yarns. In this example, however, two 150 denier yarns were weaved together as one, resulting in fill deniers of 300 and 500. The fill yarns were woven in a repeating pattern of 14 300 denier yarns followed by one 500 denier yarn. This resulted in an average fill denier of 313.33. The yarns were weaved in a plain weave with a ripstop pattern in the fill yarn.

The griuge fabric contained 41 yarns/inch in the warp and, based on the average fill denier, 47.5 yarns/inch in the fill. The density of the warp was 1,588, whereas the average density of the fill was 841.

The finished fabric contained 43 yarns/inch in the warp, 46.22 yarns/inch in the 300 denier fill, and 3.3 yarns/inch in the 500 denier fill (i.e., a total of 49.52 yarns/inch in the fill). The density of the warp was 1,665, whereas the average density of the fill was 877.

For ease of comparison, the specifications of Examples 1-3 are summarized in Tables 1 to 3.

TABLE 1

| 5 | Fabric | Weave            |                          |
|---|--------|------------------|--------------------------|
|   |        | Warp<br>(denier) | Fill<br>(average denier) |
|   | 6.11   | 500              | 157                      |
|   | 8.11   | 840              | 171.88                   |
|   | 10.11  | 1,500            | 313.33                   |

10

TABLE 2

| 15 | Fabric | Griuge Fabric                   |                 |                                 |
|----|--------|---------------------------------|-----------------|---------------------------------|
|    |        | Warp Yarn Count<br>(yarns/inch) | Warp<br>Density | Fill Yarn Count<br>(yarns/inch) |
|    | 6.11   | 62                              | 1,386           | 85                              |
|    | 8.11   | 44                              | 1,275           | 80                              |
|    | 10.11  | 41                              | 1,588           | 47.5                            |

20

TABLE 3

| 25 | Fabric | Finished Fabric                 |                 |                                 |
|----|--------|---------------------------------|-----------------|---------------------------------|
|    |        | Warp Yarn Count<br>(yarns/inch) | Warp<br>Density | Fill Yarn Count<br>(yarns/inch) |
|    | 6.11   | 75                              | 1,677           | 87.28                           |
|    | 8.11   | 55                              | 1,594           | 84                              |
|    | 10.11  | 43                              | 1,665           | 49.52                           |

30

As can be seen in Tables 1 to 3, the denier of the warp yarn was higher than that of the fill yarn in all three sailcloths. In addition, the warp yarn count was lower than the fill yarn count in all three sailcloths. The ratio of fill yarn count to warp yarn count ranged from about 1.1:1 to about 1.8:1. The warp density was higher than the fill density in all three sailcloths. The ratio of warp density to fill density ranged from about 1.2:1 to about 1.9:1.

## Example 4

This example compares the sailcloths of Examples 1-3 with other commercially available sailcloths.

The sailcloths of Examples 1-3 were compared to numerous other sailcloths, including Challenge 4.1 Radial (Challenge Sailcloth, Vernon, Conn.), Challenge 5.1 Radial (Challenge Sailcloth), Challenge 5.51 Radial (Challenge Sailcloth), Challenge 6.51 Radial (Challenge Sailcloth), Challenge 7.1 Radial (Challenge Sailcloth), Challenge 8.1 Radial (Challenge Sailcloth), Challenge 9.1 Radial (Challenge Sailcloth), Contender 5.5 Radial (Contender Sailcloth, Fall River, Mass.), Contender 6.5 Radial (Contender Sailcloth), Contender 7.5 Radial (Contender Sailcloth), Contender 8.5 Radial (Contender Sailcloth), Contender 8.01 Warp (Contender Sailcloth), Contender 5.5 Polypreg (Contender Sailcloth), Contender 6.5 Polypreg (Contender Sailcloth), Contender 7.5 Polypreg (Contender Sailcloth), Contender 8.5 Polypreg (Contender Sailcloth), Contender 9.5 Polypreg (Contender Sailcloth), Contender 10.5 Polypreg (Contender Sailcloth), Contender 9 Ultraweave (Contender Sailcloth), North 8.8 Premium Nordac (North Sails Group, Milford, Conn.), and North 12.8 (North Sails Group) sailcloths. The 1% warp, 1% fill, 1% bias, 10 lb. warp, 10 lb. fill, 10 lb. bias, 50 lb. warp, weight, and warp efficiency of each sailcloth were measured. The data are set forth in Table 4.

TABLE 4

| Sailcloth                | 1% warp | 1% fill | 1% bias | 10 lb. warp | 10 lb. fill | 10 lb. bias | 50 lb. warp | weight | warp efficiency |
|--------------------------|---------|---------|---------|-------------|-------------|-------------|-------------|--------|-----------------|
| Challenge 4.1 Radial     | 64      | 39.5    | 21.5    | 2.5         | 3.5         | 7           | 13          | 4.20   | 15.2            |
| Challenge 5.1 Radial     | 48.5    | 41      | 20      | 3.5         | 3.5         | 7           | 16.5        | 4.67   | 10.4            |
| Challenge 5.51 Radial    | 62      | 36      | 20      | 2.5         | 3.5         | 7.5         | 13.5        | 5.78   | 10.7            |
| Challenge 6.51 Radial    | 62      | 58      | 24      | 3           | 3           | 6.5         | 13.5        | 6.17   | 10.0            |
| Challenge 7.1 Radial     | 51      | 80      | 28      | 3           | 2           | 5           | 15          | 7.20   | 7.1             |
| Challenge 8.1 Radial     | 42.5    | 76      | 17.5    | 4           | 2           | 9           | 19          | 7.97   | 5.3             |
| Challenge 9.1 Radial     | 98      | 62.5    | 31.5    | 2           | 2.5         | 5           | 8.5         | 8.56   | 11.4            |
| Contender 5.5 Radial     | 35      | 52.2    | 17.09   | 4.2         | 2.52        | 8.9         | —           | 5.43   | 6.4             |
| Contender 6.5 Radial     | 53.1    | 55.54   | 26.25   | 2.84        | 2.46        | 5.74        | —           | 6.65   | 8.0             |
| Contender 7.5 Radial     | 42.3    | 53.7    | 17.3    | 4.4         | 2.6         | 9.9         | —           | 7.93   | 5.3             |
| Contender 8.5 Radial     | 47.4    | 58.6    | 16.2    | 3.86        | 2.64        | 9.74        | —           | 8.84   | 5.4             |
| Contender 9.5 Radial     | 60.7    | 60.4    | 14.4    | 3.4         | 2.6         | 11.1        | —           | 9.80   | 6.2             |
| Contender 8.01 Warp      | 59      | 20.2    | —       | 3.3         | 5.8         | 7.8         | 14.9        | 8.03   | 7.3             |
| Contender 5.5 Polypreg   | 47.6    | 42.8    | 16.6    | 3.2         | 3.1         | 9.1         | 16.9        | 4.87   | 9.8             |
| Contender 6.5 Polypreg   | 32.3    | 45.5    | 13.4    | 6.2         | 2.9         | 12          | 24          | 6.72   | 4.8             |
| Contender 7.5 Polypreg   | 54.6    | 40.3    | 19.2    | 2.8         | 3.3         | 7.8         | 14.5        | 7.21   | 7.6             |
| Contender 8.5 Polypreg   | 61.7    | 54.9    | 16.8    | 2.9         | 2.2         | 9.7         | 13          | 8.23   | 7.5             |
| Contender 9.5 Polypreg   | 40      | 58.6    | 12.1    | 6.6         | 3.1         | 13.7        | 18.8        | 9.59   | 4.2             |
| Contender 10.5 Polypreg  | 40      | 60.9    | 18.2    | 5.8         | 1.8         | 9           | 18.8        | 11.57  | 3.5             |
| Contender 9 Ultraweave   | 117     | 57.5    | 15      | 1.5         | 2.4         | 7.5         | 6.4         | 8.01   | 14.6            |
| North 8.8 Premium Nordac | 27.5    | 110     | 17.5    | 6           | 1.5         | 9           | 29.5        | 8.71   | 3.2             |
| North 12.8               | 39.5    | 164     | 23      | 4.5         | 1           | 6.5         | 10.5        | 13.20  | 3.0             |
| 6.11 (Ex. 1)             | 88      | 18      | 27      | 2           | 4.5         | 4           | 7.5         | 6.39   | 13.8            |
| 8.11 (Ex. 2)             | 140     | 10.5    | 17      | 1           | 15          | 6           | 5           | 7.94   | 17.6            |
| 10.11 (Ex. 3)            | 204     | 8.5     | 11.5    | 1.5         | 16.5        | 11          | 6.4         | 9.78   | 20.9            |

As can be seen in Table 4, while the weight of the sailcloth increases from 6.11 to 8.11 to 10.11, 1% warp and warp

of 10 lb. fill:10 lb. bias of the sailcloths were also measured. The data are set forth in Table 5.

TABLE 5

| Sailcloth                  | 1% W:1% F | 1% F:1% B | 1% W:1% F::<br>1% F:1% B | 10#W:10#F | 10#F:10#B | 10#W:10#F::<br>10#F:10#B |
|----------------------------|-----------|-----------|--------------------------|-----------|-----------|--------------------------|
| Challenge 4.1 Radial       | 1.62:1    | 1.84:1    | 0.88:1                   | 0.71:1    | 0.50:1    | 1.43:1                   |
| Challenge 5.1 Radial       | 1.18:1    | 2.05:1    | 0.58:1                   | 1:1       | 0.50:1    | 2:1                      |
| Challenge 5.51 Radial      | 1.72:1    | 1.80:1    | 0.96:1                   | 0.71:1    | 0.47:1    | 1.53:1                   |
| Challenge 6.51 Radial      | 1.07:1    | 2.42:1    | 0.44:1                   | 1:1       | 0.46:1    | 2.17:1                   |
| Challenge 7.1 Radial       | 0.64:1    | 2.86:1    | 0.22:1                   | 1.5:1     | 0.40:1    | 3.75:1                   |
| Challenge 8.1 Radial       | 0.56:1    | 4.34:1    | 0.13:1                   | 2:1       | 0.22:1    | 9:1                      |
| Challenge 9.1 Radial       | 1.57:1    | 1.98:1    | 0.79:1                   | 0.80:1    | 0.50:1    | 1.6:1                    |
| Contender 5.5 Radial       | 0.67:1    | 3.05:1    | 0.22:1                   | 1.67:1    | 0.28:1    | 5.89:1                   |
| Contender 6.5 Radial       | 0.96:1    | 2.12:1    | 0.45:1                   | 1.15:1    | 0.43:1    | 2.69:1                   |
| Contender 310 HTP-SQ Weave | 1.10:1    | 1.64:1    | 0.67:1                   | 0.76:1    | 0.66:1    | 1.15:1                   |
| Contender 7.5 Radial       | 0.79:1    | 3.10:1    | 0.25:1                   | 1.69:1    | 0.26:1    | 6.44:1                   |
| Contender 8.5 Radial       | 0.81:1    | 3.62:1    | 0.22:1                   | 1.46:1    | 0.27:1    | 5.39:1                   |
| Contender 9.5 Radial       | 1.00:1    | 4.19:1    | 0.24:1                   | 1.31:1    | 0.23:1    | 5.58:1                   |
| Contender 8.01 Warp        | 2.92:1    | —         | —                        | 0.57:1    | 0.74:1    | 0.76:1                   |
| Contender 5.5 Polypreg     | 1.11:1    | 2.58:1    | 0.43:1                   | 1.03:1    | 0.34:1    | 3.03:1                   |
| Contender 6.5 Polypreg     | 0.71:1    | 3.40:1    | 0.21:1                   | 2.14:1    | 0.24:1    | 8.85:1                   |
| Contender 7.5 Polypreg     | 1.36:1    | 2.10:1    | 0.64:1                   | 0.85:1    | 0.42:1    | 2.01:1                   |
| Contender 8.5 Polypreg     | 1.12:1    | 3.27:1    | 0.34:1                   | 1.32:1    | 0.23:1    | 5.81:1                   |
| Contender 9.5 Polypreg     | 0.68:1    | 4.84:1    | 0.14:1                   | 2.13:1    | 0.23:1    | 9.41:1                   |
| Contender 10.5 Polypreg    | 0.66:1    | 3.35:1    | 0.20:1                   | 3.22:1    | 0.20:1    | 1.61:1                   |
| Contender 9 Ultraweave     | 2.04:1    | 3.83:1    | 0.53:1                   | 0.62:1    | 0.32:1    | 1.95:1                   |
| North 8.8 Premium Nordac   | 0.25:1    | 6.29:1    | 0.04:1                   | 4:1       | 0.17:1    | 24:1                     |
| North 12.8                 | 0.24:1    | 7.13:1    | 0.03:1                   | 4.5:1     | 0.15:1    | 29.2:1                   |
| 6.11 (Ex. 1)               | 4.89:1    | 0.67:1    | 7.33:1                   | 0.44:1    | 1.12:1    | 0.39:1                   |
| 8.11 (Ex. 2)               | 13.33:1   | 0.62:1    | 21.59:1                  | 0.07:1    | 2.5:1     | 0.03:1                   |
| 10.11 (Ex. 3)              | 24:1      | 0.74:1    | 32.47:1                  | 0.09:1    | 1.5:1     | 0.06:1                   |

efficiency also increase. This finding is surprising and unexpected inasmuch as 1% warp and warp efficiency tend to remain relatively constant or decrease with increasing weight. Also, the 8.11 and 10.11 had the highest 1% warps and the highest warp efficiencies in comparison to the other sailcloths, even the lower weight sailcloths.

The ratio of 1% warp to 1% fill, the ratio of 1% fill to 1% bias, the ratio of 1% warp:1% fill to the ratio of 1% fill:1% bias, the ratio of 10 lb. warp to 10 lb. fill, the ratio of 10 lb. fill to 10 lb. bias, and the ratio of 10 lb. warp:10 lb. fill to the ratio

As can be seen in Table 5, the comparative sailcloths had a 1% warp to 1% fill ratio that ranged from 0.24:1 to 2.92:1, 60 whereas the sailcloths of the present disclosure had a 1% warp to 1% fill ratio that ranged from 4.89:1 to 24:1. The comparative sailcloths also had a 1% fill to 1% bias ratio that ranged from 1.64:1 to 7.13:1, whereas the sailcloths of the present disclosure had a 1% fill to 1% bias ratio that ranged from 0.62:1 to 0.74:1. A 1% warp:1% fill to 1% fill:1% bias ratio that ranged from 0.03 to 0.96 characterized the comparative sailcloths, whereas a 1% warp:1% fill to 1% fill:1% bias ratio 65

## 13

that ranged from 7.33:1 to 32.47:1 characterized the sailcloths of the present disclosure. The comparative sailcloths had a 10 lb. warp to 10 lb. fill ratio that ranged from 0.57:1 to 4.5:1, whereas the sailcloths of the present disclosure had a 10 lb. warp to 10 lb. fill ratio that ranged from 0.07:1 to 0.44:1. The comparative sailcloths also had a 10 lb. fill to 10 lb. bias ratio that ranged from 0.15:1 to 0.74:1, whereas the sailcloths of the present disclosure had a 10 lb. fill to 10 lb. bias ratio that ranged from 1.12:1 to 2.5:1. A 10 lb. warp:10 lb. fill to 10 lb. fill:10 lb. bias ratio that ranged from 0.76:1 to 29.2:1 characterized the comparative sailcloths, whereas a 10 lb. warp:10 lb. fill to 10 lb. fill:10 lb. bias ratio that ranged from 0.03:1 to 0.39:1 characterized the sailcloths of the present disclosure.

All patents, patent application publications, journal articles, textbooks, and other publications mentioned in the specification are indicative of the level of skill of those in the art to which the disclosure pertains. All such publications are incorporated herein by reference to the same extent as if each individual publication were specifically and individually indicated to be incorporated by reference.

The invention illustratively described herein may be suitably practiced in the absence of any element(s) or limitation(s), which is/are not specifically disclosed herein. Thus, for example, each instance herein of any of the terms "comprising," "consisting essentially of," and "consisting of" may be replaced with either of the other two terms. Likewise, the singular forms "a," "an," and "the" include plural references unless the context clearly dictates otherwise. Thus, for example, references to "the method" includes one or more methods and/or steps of the type, which are described herein and/or which will become apparent to those ordinarily skilled in the art upon reading the disclosure.

The terms and expressions, which have been employed, are used as terms of description and not of limitation. In this regard, where certain terms are defined at the beginning of the "Detailed Description" and are otherwise defined, described, or discussed elsewhere in the disclosure, all such definitions, descriptions, and discussions are intended to be attributed to such terms. There also is no intention in the use of such terms and expressions of excluding any equivalents of the features shown and described or portions thereof.

It is recognized that various modifications are possible within the scope of the claimed invention. Thus, it should be understood that, although the present invention has been specifically disclosed in the context of preferred embodiments and optional features, those skilled in the art may resort to modifications and variations of the concepts disclosed herein. Such modifications and variations are considered to be within the scope of the invention as defined by the appended claims.

What is claimed is:

1. A woven sailcloth comprising warp yarns and fill yarns and having a 1% warp of at least about 125 and/or a warp efficiency of at least about 17.

2. The woven sailcloth of claim 1, which also has a weight of at least about 7.

3. The woven sailcloth of claim 1, which has a 1% warp of at least about 190 and/or a warp efficiency of at least about 21.

4. The woven sailcloth of claim 3, which also has a weight of at least about 9.

5. The woven sailcloth of claim 1, which also has at least one of:

- (a) a 1% warp to 1% fill ratio of at least about 4:1,
- (b) a 1% fill to 1% bias ratio of less than about 1:1,
- (c) a 1% warp:1% fill to 1% fill:1% bias ratio of at least about 1:1,
- (d) a 10 lb. warp to 10 lb. fill ratio of less than about 0.5:1,
- (e) a 10 lb. fill to 10 lb. bias ratio of at least about 1:1, and

## 14

(f) a 10 lb. warp:10 lb. fill to 10 lb. fill:10 lb. bias ratio of less than about 0.5:1.

6. The woven sailcloth of claim 1, wherein the fill yarns are pre-crimped.

7. The woven sailcloth of claim 1, wherein the warp yarns and the fill yarns are weaved in a plain weave in which the ratio of fill yarn count to warp yarn count is about 1.1:1 to about 1.8:1 and the ratio of warp yarn density to fill yarn density is about 1.2:1 to about 1.9:1.

8. The woven sailcloth of claim 7, wherein the fill yarns comprise a reinforcing yarn.

9. The woven sailcloth of claim 8, wherein the reinforcing yarn is present every  $n^{th}$  yarn, wherein  $n$  is an integer from and including 5 to and including 20.

10. The woven sailcloth of claim 9, wherein the fill yarns are weaved in a ripstop pattern.

11. A woven sailcloth comprising warp yarns and fill yarns weaved in a plain weave in which the ratio of fill yarn count to warp yarn count is about 1.1:1 to about 1.8:1 and the ratio of warp yarn density to fill yarn density is about 1.2:1 to about 1.9:1, wherein the woven sailcloth has a 1% warp of at least about 125 and/or a warp efficiency of at least about 17.

12. The woven sailcloth of claim 11, which has a weight of at least about 7.

13. The woven sailcloth of claim 11, which has a 1% warp of at least about 190 and/or a warp efficiency of at least about 21.

14. The woven sailcloth of claim 13, which has a weight of at least about 9.

15. The woven sailcloth of claim 11, which has at least one of:

- (a) a 1% warp to 1% fill ratio of at least about 4:1,
- (b) a 1% fill to 1% bias ratio of less than about 1:1,
- (c) a 1% warp:1% fill to 1% fill:1% bias ratio of at least about 1:1,
- (d) a 10 lb. warp to 10 lb. fill ratio of less than about 0.5:1,
- (e) a 10 lb. fill to 10 lb. bias ratio of at least about 1:1, and
- (f) a 10 lb. warp:10 lb. fill to 10 lb. fill:10 lb. bias ratio of less than about 0.5:1.

16. The woven sailcloth of claim 11, wherein the fill yarns are pre-crimped.

17. The woven sailcloth of claim 11, wherein the fill yarns comprise a reinforcing yarn.

18. The woven sailcloth of claim 17, wherein the reinforcing yarn is present every  $n^{th}$  yarn, wherein  $n$  is an integer from and including 5 to and including 20.

19. The woven sailcloth of claim 18, wherein the fill yarns are weaved in a ripstop pattern.

20. A woven sailcloth comprising warp yarns and fill yarns and having a weight of at least about 7 and at least one of:

- (a) a 1% warp to 1% fill ratio of at least about 4:1,
- (b) a 1% fill to 1% bias ratio of less than about 1:1,
- (c) a 1% warp:1% fill to 1% fill:1% bias ratio of at least about 1:1,
- (d) a 10 lb. warp to 10 lb. fill ratio of less than about 0.5:1,
- (e) a 10 lb. fill to 10 lb. bias ratio of at least about 1:1, and
- (f) a 10 lb. warp:10 lb. fill to 10 lb. fill:10 lb. bias ratio of less than about 0.5:1.

21. The woven sailcloth of claim 20, which has a 1% warp of at least about 125 and/or a warp efficiency of at least about 17.

22. The woven sailcloth of claim 20, which has a 1% warp of at least about 190 and/or a warp efficiency of at least about 21.

23. The woven sailcloth of claim 22, which has a weight of at least about 9.

## 15

24. The woven sailcloth of claim 20, wherein the fill yarns are pre-crimped.

25. The woven sailcloth of claim 20, wherein the warp yarns and the fill yarns are weaved in a plain weave in which the ratio of fill yarn count to warp yarn count is about 1.1:1 to about 1.8:1 and the ratio of warp yarn density to fill yarn density is about 1.2:1 to about 1.9:1.

26. The woven sailcloth of claim 25, wherein the fill yarns comprise a reinforcing yarn.

27. The woven sailcloth of claim 26, wherein the reinforcing yarn is present every  $n^{th}$  yarn, wherein  $n$  is an integer from and including 5 to and including 20.

28. The woven sailcloth of claim 27, wherein the fill yarns are weaved in a ripstop pattern.

29. A woven sailcloth having a weight of at least about 7 and comprising warp yarns and fill yarns weaved in a plain weave in which the ratio of fill yarn count to warp yarn count is about 1.1:1 to about 1.8:1 and the ratio of warp yarn density to fill yarn density is about 1.2:1 to about 1.9:1, wherein the woven sailcloth has a 1% warp of at least about 125 and/or a warp efficiency of at least about 17, and wherein the woven sailcloth has at least one of a 1% warp to 1% fill ratio of at least about 4:1, a 1% fill to 1% bias ratio of less than about 1:1, a 1% warp : 1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1.

30. The woven sailcloth of claim 29, wherein the weight of the sailcloth is at least about 9, the 1% warp is at least about 190 and the warp efficiency is at least about 21.

31. A sail comprising at least one panel of the woven sailcloth of claim 29, wherein the at least one panel of the woven sailcloth is assembled into the sail with load paths oriented along its warp yarns.

32. A sail comprising at least one panel of the woven sailcloth of claim 30, wherein the at least one panel of the woven sailcloth is assembled into the sail with load paths oriented along its warp yarns.

33. A sail comprising at least one panel of the woven sailcloth of claim 11, wherein the at least one panel of the woven sailcloth is assembled into the sail with load paths oriented along its warp yarns.

34. A sail comprising at least one panel of the woven sailcloth of claim 12, wherein the at least one panel of the woven sailcloth is assembled into the sail with load paths oriented along its warp yarns.

35. A sail comprising at least one panel of the woven sailcloth of claim 13, wherein the at least one panel of the woven sailcloth is assembled into the sail with load paths oriented along its warp yarns.

36. A sail comprising at least one panel of the woven sailcloth of claim 14, wherein the at least one panel of the woven sailcloth is assembled into the sail with load paths oriented along its warp yarns.

37. A sail comprising at least one panel of the woven sailcloth of claim 15, wherein the at least one panel of the woven sailcloth is assembled into the sail with load paths oriented along its warp yarns.

38. A sail comprising at least one panel of the woven sailcloth of claim 20, wherein the at least one panel of the woven sailcloth is assembled into the sail with load paths oriented along its warp yarns.

39. A sail comprising at least one panel of the woven sailcloth of claim 21, wherein the at least one panel of the woven sailcloth is assembled into the sail with load paths oriented along its warp yarns.

## 16

40. A sail comprising at least one panel of the woven sailcloth of claim 22, wherein the at least one panel of the woven sailcloth is assembled into the sail with load paths oriented along its warp yarns.

41. A sail comprising at least one panel of the woven sailcloth of claim 23, wherein the at least one panel of the woven sailcloth is assembled into the sail with load paths oriented along its warp yarns.

42. A sail comprising at least one panel of the woven sailcloth of claim 25, wherein the at least one panel of the woven sailcloth is assembled into the sail with load paths oriented along its warp yarns.

43. A method of making a woven sailcloth comprising warp yarns and fill yarns, which method comprises weaving warp yarns and fill yarns in a plain weave in which the ratio of fill yarn count to warp yarn count is about 1.1:1 to about 1.8:1 and the ratio of warp yarn density to fill yarn density is about 1.2:1 to about 1.9:1, whereupon a woven sailcloth comprising warp yarns and fill yarns is made.

44. The method of claim 43, wherein the fill yarns are pre-crimped.

45. The method of claim 43, wherein the fill yarns comprise a reinforcing yarn.

46. The method of claim 45, wherein the reinforcing yarn is present every  $n^{th}$  yarn, wherein  $n$  is an integer from and including 5 to and including 20.

47. The method of claim 46, wherein the fill yarns are weaved in a ripstop pattern.

48. A method of making a sail, which method comprises assembling panels of sailcloth, at least one panel of which is woven sailcloth comprising warp yarns and fill yarns and having a 1% warp of at least about 125 and/or a warp efficiency of at least about 17, wherein the at least one panel of woven sailcloth is assembled into the sail with load paths oriented along its warp yarns, whereupon a sail is made.

49. The method of claim 48, wherein the at least one panel of woven sailcloth has a 1% warp of at least about 190 and/or a warp efficiency of at least about 21.

50. The method of claim 48, wherein the at least one panel of woven sailcloth also has at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1.

51. The method of claim 48, wherein the at least one panel of woven sailcloth has a ratio of fill yarn count to warp yarn count of about 1.1:1 to about 1.8:1 and a ratio of warp yarn density to fill yarn density of about 1.2:1 to about 1.9:1.

52. A method of making a sail, which method comprises assembling panels of sailcloth, at least one panel of which is woven sailcloth comprising warp yarns and fill yarns weaved in a plain weave in which the ratio of fill yarn count to warp yarn count is about 1.1:1 to about 1.8:1 and the ratio of warp yarn density to fill yarn density is about 1.2:1 to about 1.9:1, wherein the woven sailcloth has a 1% warp of at least about 125 and/or a warp efficiency of at least about 17, whereupon a sail is made.

53. The method of claim 52, wherein the woven sailcloth has a weight of at least about 7.

54. The method of claim 52, wherein the woven sailcloth has a 1% warp of at least about 190 and/or a warp efficiency of at least about 21.

55. The method of claim 54, wherein the woven sailcloth has a weight of at least about 9.

**56.** The method of claim **52**, wherein the woven sailcloth has at least one of:

- (a) a 1% warp to 1% fill ratio of at least about 4:1,
- (b) a 1% fill to 1% bias ratio of less than about 1:1,
- (c) a 1% warp:1% fill to 1% fill:1% bias ratio of at least about 1:1,
- (d) a 10 lb. warp to 10 lb. fill ratio of less than about 0.5:1,
- (e) a 10 lb. fill to 10 lb. bias ratio of at least about 1:1, and
- (f) a 10 lb. warp:10 lb. fill to 10 lb. fill:10 lb. bias ratio of less than about 0.5:1.

**57.** A method of making a sail, which method comprises assembling panels of sailcloth, at least one panel of which is woven sailcloth having a weight of at least about 7 and comprising warp yarns and fill yarns, wherein (i) the at least one panel of woven sailcloth has at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, a 10 lb. warp:10 lb. fill to 10 lb. fill:10 lb. bias ratio of less than about 0.5:1 and (ii) the at least one panel of woven sailcloth is assembled into the sail with load paths oriented along its warp yarns, whereupon a sail is made.

**58.** The method of claim **57**, wherein the at least one panel of woven sailcloth also has a 1% warp of at least about 125 and/or a warp efficiency of at least about 17.

**59.** The method of claim **57**, wherein the at least one panel of woven sailcloth also has a 1% warp of at least about 190 and/or a warp efficiency of at least about 21.

**60.** The method of claim **57**, in which the ratio of fill yarn count to warp yarn count is about 1.1:1 to about 1.8:1 and the ratio of warp yarn density to fill yarn density is about 1.2:1 to about 1.9:1.

**61.** A method of making a sail, which method comprises assembling panels of sailcloth, at least one of which is a panel of woven sailcloth having a weight of at least about 7 and comprising warp yarns and fill yarns weaved in a plain weave in which the ratio of fill yarn count to warp yarn count is about 1.1:1 to about 1.8:1 and the ratio of warp yarn density to fill yarn density is about 1.2:1 to about 1.9:1, wherein the woven sailcloth has a 1% warp of at least about 125, a warp efficiency of at least about 17, and at least one of a 1% warp to 1% fill ratio of at least about 4:1, a 1% fill to 1% bias ratio of less than about 1:1, a 1% warp:1% fill to 1% fill:1% bias ratio of at least about 1:1, a 10 lb. warp to 10 lb. fill ratio of less than about 0.5:1, a 10 lb. fill to 10 lb. bias ratio of at least about 1:1, and a 10 lb. warp:10 lb. fill to 10 lb. fill:10 lb. bias ratio of less than about 0.5:1, whereupon a sail is made.

**62.** The method of claim **61**, wherein the weight of the woven sailcloth is at least about 9, the 1% warp is at least about 190 and the warp efficiency is at least about 21.

\* \* \* \* \*